

1

3,498,857  
ALUMINUM-IRON OXIDE INCENDIARY COMPOSITION CONTAINING A (CYCLOPENTADIENYL) IRON COMPOUND

Urho Albert Lehtikoinen, Detroit, Mich., assignor to Ethyl Corporation, New York, N.Y., a corporation of Virginia  
No Drawing. Filed Dec. 6, 1966, Ser. No. 600,006

Int. Cl. C06b 1/00

U.S. Cl. 149—21

11 Claims

### ABSTRACT OF THE DISCLOSURE

Bis(cyclopentadienyl)iron and bis(alkylcyclopentadienyl)iron compounds (also known as ferrocene-type compounds) improve the ignition and burning properties of thermites and thermates. Preferred thermites are composed of powdered aluminum and an iron oxide. In addition to these ingredients, the thermates contain materials such as flake aluminum, sulfur, hydrocarbon oils, and oxidizers such as barium nitrate. The improved compositions are useful in incendiary weapons, as munitions or as starters for other pyrotechnic materials.

This invention relates to improved pyrotechnic compositions for incendiary munitions. More specifically, the improvement relates to compositions known as thermites and thermates.

Typically, thermites are mixtures of powdered aluminum and iron oxide. Broadly speaking, however, thermites may also be mixtures of magnesium and iron oxide, zirconium and iron oxide, and the like. Upon ignition, thermites undergo strongly exothermic reactions. For example, magnetite reacts with aluminum as follows:



Red iron oxide,  $\text{Fe}_2\text{O}_3$ , reacts with aluminum in a similar manner. Therefore, it may also be employed in thermites. These reactions are well-known in the art.

Generally, thermites have a major deficiency; they are not readily ignitable. Various additives which decrease the ignition temperature are known in the art. Thermites modified with these additives are in military use and are called thermates. Thus, typical thermates contain metal-metal oxide systems such as those mentioned above and, in addition, contain oxidizers such as barium nitrate, potassium chromate and potassium permanganate. Other components used in thermates are sulfur, hydrocarbon oils, zinc powder, magnesium powder, and the like. Although these additives somewhat lower the ignition temperature and accelerate burning, the improvement is only partial and not totally satisfactory.

Since thermites and thermates presently available are often unsatisfactory, an object of this invention is to prepare said materials having superior igniting and burning properties. Further objects will be apparent from the following detailed description and appended claims.

The objects of this invention are accomplished by incorporating in conventional thermites and thermates one or more compounds having the following general formula:

2



wherein  $R_1$  to  $R_4$  are the same or different and can be hydrogen or an alkyl group having up to six carbon atoms. Said aliphatic groups can be straight or branched chains and can have one or more olefinic bonds. Non-limiting examples of compounds described by the above general formula are bis(cyclopentadienyl)iron, (cyclopentadienyl)(methylcyclopentadienyl)iron, (cyclopentadienyl)(ethylcyclopentadienyl)iron, bis(propylcyclopentadienyl)iron, bis(isopropylcyclopentadienyl)iron, bis(butylcyclopentadienyl)iron, bis(tert - butylcyclopentadienyl)iron, bis(hexylcyclopentadienyl)iron, bis(methylcyclopentadienyl)iron, (cyclopentadienyl)(dimethylcyclopentadienyl)iron, bis(ethylcyclopentadienyl)iron, and (cyclopentadienyl)(diethylcyclopentadienyl)iron, and the like. The above compounds, also known as ferrocene-type compounds, illustrate that both symmetrical and unsymmetrical alkyl ferrocenes may be employed. By symmetrical and unsymmetrical is meant alkyl ferrocenes with heteroannular and homoannular substitution respectively. Ferrocene and alkyl ferrocene polymers may also be employed in this invention.

The most preferred compounds defined by the above formula are bis(cyclopentadienyl)iron and the alkyl derivatives thereof having 11 to 14 carbon atoms, such as (cyclopentadienyl)(methylcyclopentadienyl)iron, bis(methylcyclopentadienyl)iron and (cyclopentadienyl)(dimethylcyclopentadienyl)iron, (cyclopentadienyl)(ethylcyclopentadienyl)iron, bis(ethylcyclopentadienyl)iron, and (cyclopentadienyl)(diethylcyclopentadienyl)iron.

Any ignition and combustion-improving amount of a ferrocene-type compound may be incorporated in thermites and thermates of this invention, although 2 to 50 weight percent of the total composition is generally found to be adequate. A more preferred amount of a ferrocene-type compound is from about 10 to about 35 weight percent of the total composition.

The improvement of ignition and burning properties of thermites and thermates is illustrated in Table 1 below. Table 1 shows how ignition and combustion properties of various compositions were consistently improved when ferrocene was added. Every example in Table 1 shows the results obtained when a pyrotechnic material in a powdered form was wetted with toluene and thereafter ignited. Magnesium ribbon is generally employed as a starter for thermites and thermates. However, toluene was used as a starter in the tests reported in Table 1 because of convenience. Each example demonstrates the improved ignition and combustion properties obtained when the specified amount of bis(cyclopentadienyl)iron (ferrocene) was added to the pyrotechnic composition first tested without ferrocene. The thermite employed in the pyrotechnics reported in Table 1 had the following composition: aluminum, 25.2 weight percent, and iron oxide ( $\text{Fe}_2\text{O}_3$ ), 74.8 weight percent.

TABLE 1.—IGNITION AND COMBUSTION OF POWDERED THERMITE AND THERMATE COMPOSITIONS

| Example No. | Composition, parts by weight |                                 |                                   |           |                   |                | Comments                                                            |
|-------------|------------------------------|---------------------------------|-----------------------------------|-----------|-------------------|----------------|---------------------------------------------------------------------|
|             | Thermite                     | K <sub>2</sub> CrO <sub>4</sub> | Ba(NO <sub>3</sub> ) <sub>2</sub> | Ferrocene | Aluminum<br>flake | Zinc<br>powder |                                                                     |
| 1.....      | 1.....                       | 1.....                          | 1.....                            | 1.....    | 1.....            | 1.....         | Did not burn.<br>Brief flare. Very little material burned.          |
| 2.....      | 1.....                       | 1.....                          | 1.....                            | 1.....    | 1.....            | 1.....         | Did not burn.<br>Small flares. Very little material burned.         |
| 3.....      | 1.....                       | 1.....                          | 1.....                            | 1.....    | 1.....            | 1.....         | Did not burn.<br>Burned completely.<br>About 85% of charge burned.  |
| 4.....      | 1.....                       | 1.....                          | 1.....                            | 1.....    | 1.....            | 1.....         | Did not burn.<br>About 30% of charge burned.                        |
| 5.....      | 1.....                       | 1.....                          | 1.....                            | 1.....    | 1.....            | 1.....         | 1 Did not burn.<br>1 Burned completely.                             |
| 6.....      | 0.7.....                     | 0.3.....                        | 0.3.....                          | 1.....    | 1.....            | 1.....         | Brief flare-ups, very little burned.<br>About 50% of charge burned. |

In the above examples, analytical grade crystalline Ba(NO<sub>3</sub>)<sub>2</sub> was employed.

Similar results are obtained when, in the above examples, (cyclopentadienyl)(methylcyclopentadienyl)iron, (cyclopentadienyl)(hexylcyclopentadienyl)iron, bis(propylcyclopentadienyl)iron, bis(tert-butylcyclopentadienyl)iron, and bis(methylcyclopentadienyl)iron and (cyclopentadienyl)(dimethylcyclopentadienyl)iron are substituted for bis(cyclopentadienyl)iron (ferrocene).

The above table, thus, clearly shows that the ignition of the compositions containing ferrocene-type compounds is improved and that the burning of these compositions is much more complete. The improvement of the ignition and burning properties attributed to ferrocene is more outstanding in pelletized thermates as shown in Example 7 below.

#### EXAMPLE 7

Two pyrotechnic compositions were prepared separately. One was the thermite composition employed in Table 1, above, having 25.2 weight percent of powdered aluminum and 74.8 percent of iron oxide (Fe<sub>2</sub>O<sub>3</sub>). The other composition contained one part by weight of the above-mentioned thermite, one part by weight of potassium permanganate, one part by weight ferrocene, and 0.5 part by weight zinc powder. Solid pellets (1/2" O.D., 3/16" thick) were prepared in such a manner that one-half of each pellet consisted of the thermite composition and the other half consisted of the thermate composition containing ferrocene. The pellets were wetted with toluene and ignited. The portion of each pellet consisting of the ferrocene-containing thermate composition ignited immediately and burned completely. However, the thermite portion of the pellet which did not contain ferrocene did not burn at all.

Table 2 below shows the improved ignition and burning properties of additional thermates containing ferrocene. These thermates have been pelletized to form hollow-core pellets (1/16" O.D., 1/16" I.D., 1/16" thick). The pellets were saturated with toluene and ignited. The composition of the thermite employed in the thermates reported in Table 2 was the same as that employed in the thermates reported in Table 1.

Similar results are obtained when, in Examples 7 to 10, (cyclopentadienyl)(methylcyclopentadienyl)iron, (cyclopentadienyl)(ethylcyclopentadienyl)iron, bis(propylcyclopentadienyl)iron, bis(tert-butylcyclopentadienyl)iron, and bis(methylcyclopentadienyl)iron and (cyclopentadienyl)(dimethylcyclopentadienyl)iron are substituted for bis(cyclopentadienyl)iron (ferrocene).

Considering the fact that even finely divided thermates which have a large surface area are not easily ignited, it is most startling that pelletized thermates, which have a very small surface area, can be ignited and burned with such ease as demonstrated in Example 7 and in Table 2 above.

Thermates and thermites improved by the addition of ferrocene-type compounds may be employed in the same manner and for the same purposes as conventional thermates. The most widely known uses of thermates and thermites are as incendiary materials in munitions or as starters for other incendiary materials which are more difficult to ignite. An example of said use is in a magnesium aerial bomb which is filled with a thermite or a thermate. Another example of the use of the compositions of this invention is in napalms. More specifically, a napalm having the following composition would be useful in military applications: 35 weight percent of a pelletized thermate composed of 1 part by weight of a thermite (74.8 wt. percent of Fe<sub>2</sub>O<sub>3</sub> and 25.2 wt. percent of powdered aluminum), 1 part by weight of potassium permanganate and 1 part by weight of ferrocene; dispersed in 65 weight percent of conventional napalm (gasoline gelled in soap or heavy metal soap mixtures).

It was stated above that, in the tests reported in the preceding examples, toluene was employed as a starter. The thermite and thermate compositions of this invention exhibit the same improved incendiary properties when starters generally employed in military applications, such as magnesium ribbon, are used.

Having fully disclosed the novel composition and processes of this invention and their use, it is desired that this invention be limited only within the lawful scope of the appended claims.

I claim:

1. In a pyrotechnic composition selected from the group consisting of iron oxide-aluminum based thermites and thermates, the improvement consisting essentially of the addition of two to 50 weight percent of the total

TABLE 2

| Example No. | Parts by weight |                   |           |                                                               |
|-------------|-----------------|-------------------|-----------|---------------------------------------------------------------|
|             | Thermite        | KMnO <sub>4</sub> | Ferrocene | Comments                                                      |
| 8.....      | 1.....          | 1.....            | 0.5.....  | Ignited and burned completely. Burning time, 3 seconds.       |
| 9.....      | 1.....          | 1.....            | 0.25..... | Ignited and burned completely. Burning time, 1 second.        |
| 10.....     | 1.....          | 1.....            | 1.0.....  | Ignited and burned completely. Burning time, -5 to 7 seconds. |

composition of an ignition-improving compound having the general formula:



wherein R<sub>1</sub>, R<sub>2</sub>, R<sub>3</sub>, and R<sub>4</sub> are independently selected from the group consisting of hydrogen and alkyl groups having up to six carbon atoms. 10

2. The composition of claim 1 wherein said ignition-improving compound is selected from the group consisting of bis(cyclopentadienyl)iron, (cyclopentadienyl)(methylcyclopentadienyl)iron, (cyclopentadienyl)(ethylcyclopentadienyl)iron, bis(methylcyclopentadienyl)iron, (cyclopentadienyl)(dimethylcyclopentadienyl) iron, bis(ethylcyclopentadienyl)iron, and cyclopentadienyl(dimethylcyclopentadienyl)iron. 15

3. The composition of claim 2 wherein the amount of 20 said ignition-improving compound is from about 10 to about 35 weight percent of the total composition.

4. A thermite composition of claim 1 wherein said thermite comprises 25 to 28 weight percent of powdered aluminum and 72 to 75 weight percent of an iron oxide 25 selected from the group consisting of magnetite, Fe<sub>3</sub>O<sub>4</sub>, and red iron oxide, Fe<sub>2</sub>O<sub>3</sub>.

5. The composition of claim 4 wherein said ignition-improving compound is selected from the group consisting of bis(cyclopentadienyl)iron, (cyclopentadienyl)(methylcyclopentadienyl)iron, (cyclopentadienyl)(ethylcyclopentadienyl)iron, bis(methylcyclopentadienyl)iron, (cyclopentadienyl)(dimethylcyclopentadienyl) iron, bis(ethylcyclopentadienyl)iron, and (cyclopentadienyl)(diethylcyclopentadienyl)iron. 30

6. The composition of claim 4 wherein said ignition-improving compound is bis(cyclopentadienyl)iron.

7. The composition of claim 5 wherein the amount of 35 said ignition-improving compound is from about 10 to about 35 weight percent of the total composition.

8. The composition of claim 1 wherein said thermite comprises

60 to 80 weight percent of a thermite containing 25 to 28 weight percent of aluminum powder and 72 to 75 weight percent of an iron oxide, 0 to 4 weight percent of flake aluminum, 0 to 5 weight percent of sulfur, 10 to 30 weight percent of an oxidizer selected from the group consisting of barium nitrate, potassium permanganate, and potassium chromate, 0 to 10 weight percent of zinc powder, and 0 to 10 weight percent of magnesium powder.

9. The composition of claim 7 wherein said ignition-improving compound is selected from the group consisting of bis(cyclopentadienyl)iron, (cyclopentadienyl)(methylcyclopentadienyl)iron, (cyclopentadienyl)(ethylcyclopentadienyl)iron, bis(methylcyclopentadienyl)iron, (cyclopentadienyl)(dimethylcyclopentadienyl) iron, bis(ethylcyclopentadienyl)iron, and (cyclopentadienyl)(diethylcyclopentadienyl)iron.

10. The composition of claim 8 wherein the amount of 20 said ignition-improving compound is from about 10 to about 35 weight percent of the total composition.

11. The composition of claim 10 wherein said ignition-improving compound is bis(cyclopentadienyl)iron.

#### References Cited

##### UNITED STATES PATENTS

|           |        |                 |        |    |
|-----------|--------|-----------------|--------|----|
| 3,254,996 | 6/1966 | MacDonald       | 149—37 | XR |
| 3,297,503 | 1/1967 | Hoffmann et al. | 149—37 | XR |
| 3,309,249 | 3/1967 | Allen           | 149—37 | XR |
| 3,325,316 | 6/1967 | MacDonald       | 149—37 | XR |
| 3,344,210 | 9/1967 | Silvia          | 149—37 | XR |

35 C. D. QUARFORTH, Primary Examiner  
S. J. LECHERT, Jr., Assistant Examiner

U.S. CL. X.R.

40 149—41, 43 44, 61